

## UNITED STATES PATENT OFFICE

CHARLES HENRY PROCTOR, OF ARLINGTON, NEW JERSEY, ASSIGNOR TO THE ROESSLER & HASSLACHER CHEMICAL COMPANY, OF NEW YORK, N. Y., A CORPORATION OF NEW YORK

## ELECTRODEPOSITION OF CHROMIUM

No Drawing.

Application filed March 9, 1929. Serial No. 345,888.

This invention relates to improvements in the electrodeposition of chromium.

The electrolytic baths commonly used for plating articles with chromium contain chromic acid and usually include small amounts of sulphate ions. A great variety of addition agents, such as inorganic salts, have been dissolved with the chromic acid in the prior art baths. However, a limitation of these baths is that they do not "throw" a deposit into the recesses of irregularly shaped articles which are being chromium plated.

I have now found that the presence of a naturally occurring chrome-iron ore, such as chromite, in electrolytic solutions containing chromic acid shortens the time in which deposits can be plated out. The resulting deposits are also whiter and more evenly distributed over the object to be plated than those which have been obtained by the chromic acid baths previously known.

My invention also increases the throwing power of chromic acid baths, shortens the time in which good deposits will begin to appear, and the internal resistance of the baths is less than that of the previously known chromic acid baths.

Chrome-iron ores are known to contain in general the following oxides in approximately the proportions given:

Chromic oxide ( $\text{Cr}_2\text{O}_3$ )----- 45-65%  
Iron oxides ( $\text{Fe}_2\text{O}_3$ )----- 20-35%  
Magnesium oxide ( $\text{MgO}$ )----- 4-16%  
Aluminum oxide ( $\text{Al}_2\text{O}_3$ )----- 7-20%  
Silicon dioxide ( $\text{SiO}_2$ )----- 4-7%

The naturally occurring chrome-iron ore, which I prefer to dissolve in my baths, can be obtained commercially in the form of a fine powder, the empirical formula of which shows essentially the following oxides or their equivalents in about the proportions given:

By weight  
Chromic oxide ( $\text{Cr}_2\text{O}_3$ )----- 48-50%  
Iron oxides ( $\text{Fe}_2\text{O}_3$ )----- 20-25%  
Silicon oxide ( $\text{SiO}_2$ )----- 4-7%  
Magnesium oxide ( $\text{MgO}$ )----- 12-14%  
Aluminum oxide ( $\text{Al}_2\text{O}_3$ )----- 7-10%

One example of my successful chromic acid baths is as follows:

|                                           |                                     |
|-------------------------------------------|-------------------------------------|
| Water-----                                | 1 gallon                            |
| Chromic acid-----                         | 8-48 oz. 55                         |
| Chrome-iron ore----- (as described above) | $\frac{1}{4}$ to $1\frac{1}{2}$ oz. |
| Sulphuric acid (60%)-----                 | $\frac{1}{2}$ to $\frac{1}{2}$ oz.  |

Anodes of sheet steel or lead may be used and the bath temperature maintained at 95-120° F. with current densities of 100-125 amps. per sq. ft.

What I claim is:

1. As a new composition, a chromic acid electroplating solution containing chrome-iron ore. 65
2. As a new composition a chromic acid electroplating solution containing, for each gallon of water, the following ingredients in about the proportions given: 70

|                                      |                                        |
|--------------------------------------|----------------------------------------|
| Chromic acid ( $\text{CrO}_3$ )----- | 8 to 48 ozs.                           |
| Chrome-iron ore (commercial)-----    | $\frac{1}{4}$ to $1\frac{1}{2}$ ozs.   |
| Sulfuric acid-----                   | $\frac{1}{2}$ to $\frac{1}{2}$ ozs. 75 |

the chrome-iron ore having essentially the following analysis:

|                                                 | By weight |
|-------------------------------------------------|-----------|
| Chrome oxide ( $\text{Cr}_2\text{O}_3$ )-----   | 48-50% 80 |
| Iron oxide ( $\text{Fe}_2\text{O}_3$ )-----     | 20-25%    |
| Silicon oxide ( $\text{SiO}_2$ )-----           | 4-7%      |
| Magnesium oxide ( $\text{MgO}$ )-----           | 12-14%    |
| Aluminum oxide ( $\text{Al}_2\text{O}_3$ )----- | 7-10%     |

Signed at New York city, N. Y., in the county of New York and State of New York this 16th day of February, A. D. 1929.

CHARLES HENRY PROCTOR.

90

95